

# UNITED STATES PATENT OFFICE.

WILLIAM H. JONES, OF MUNHALL, AND ANDREW F. MITCHELL, OF HOMESTEAD, PENNSYLVANIA.

## PROCESS OF TREATING STEEL AND STEEL ALLOYS.

1,076,768.

Specification of Letters Patent.

Patented Oct. 28, 1913.

No Drawing.

Application filed February 4, 1911. Serial No. 606,591.

*To all whom it may concern:*

Be it known that we, WILLIAM H. JONES, of Munhall, and ANDREW F. MITCHELL, of Homestead, in the county of Allegheny and State of Pennsylvania, have invented certain new and useful Improvements in Processes of Treating Steel and Steel Alloys, of which the following is a full, clear, and exact description.

10 Our invention relates to the treatment of steel and steel alloys which have been shaped or partly shaped from the ingot into which the molten metal is cast and the invention is designed to provide an improved method 15 of treating the steel whereby its structure is changed and the strength and toughness of the hardened steel are increased.

One method heretofore used for treating steel to increase its hardness and toughness 20 is to super-carburize part or the whole of the perimetric surface of the steel and then harden by heating and water quenching the steel. When such super-carburized steel is afterward hardened the super-carburized 25 portion of the steel has a coarse crystalline structure so extremely brittle that the outer surface is easily cracked and liable to flake off or spawl when subjected to the uses for which the steel is intended.

30 One object of our invention is to provide a novel method of treating steel such as is used in making rolls for rolling mills, die blocks, rolls used in cold rolling other steel, race rings for roller and ball bearings, 35 and steel articles generally requiring an extremely hard outer or wearing surface formed integral with a relatively soft tougher interior or back, and the disadvantages above described thereby avoided 40 and overcome.

In the practice of our improved method, steel or a steel alloy of the desired composition is first super-carburized by any of the various well-known super-carburizing methods. By means of this operation, steel containing, say .30 per cent. carbon is super-carburized so as to obtain about 1.5 per cent. of carbon on the outer surface or the desired part of such outer surface of the steel. This 50 super-carburization extends inwardly from a maximum amount at the outer surface to a depth of about one and one half inches, more or less, from the surface, the amount of carbon present gradually decreasing inwardly until the original carbon content of

the steel before recarburizing is reached. In the second or decarburizing step of our improved method, such super-carburized steel is then decarburized on its outer surface, the depth to which the decarburizing operation 60 extends varying according to the decarburizing agent used and the length of time the decarburizing operation is continued. The steel, which preferably has been super-carburized on the desired portions of its outer 65 surface in accordance with the above described method, is decarburized by placing the steel within a box of suitable refractory material with the surface or surfaces to be decarburized adjacent to or resting upon a 70 bed of silica sand or finely ground iron ore, and is heated to a temperature approximating 1025 degrees centigrade for a varying length of time (from two to eight days) depending upon the depth to which the decarburizing is to be effected. In this operation, the surface of the metal will be decarburized to the point where it is practically free from or very low in carbon and in accordance 75 with our method the steel may originally 80 be made of such thickness or diameter as to allow this outer surface to be removed by machining, after the decarburizing operation is completed. In this way the very soft decarburized surface will be removed and 85 the new surface thus obtained will have a carbon content of from .60 to .80 per cent., this amount of carbon being sufficient to afford a hard wearing surface after being later subjected to the hardening operation. 90

Another way of providing the desired carbon content of from .60 to .80 per cent. at the surface of the steel after decarburizing, is to again inclose the steel within a covering of suitable refractory material, after 95 covering the decarburized surface with a mild recarburizing agent, and then heat the steel to a temperature of about 975 degrees centigrade for a period of from about 10 to as high as 24 hours, in this way recarburizing or again increasing the carbon content of the outer surface to the desired extent. 100

After the decarburized portions of the super-carburized steel have been treated, either by machining to remove the outer decarburized surface, or by recarburizing to increase the carbon content of the decarburized surface, the steel is then tempered or hardened by heating and quenching in water, oil or other cooling medium in the usual 110

manner, this operation providing the outer surface of the steel with a very hard wearing surface of fine, clear chill structure similar to that of tool steel, which is joined to the soft tough portion of interior having a fibrous structure. In some cases the steel may be heated and quenched in water in order to harden after the completion of the decarburization of the supercarburized face 10 and the step of removing part of the decarburized face portion omitted. In this way a steel having two distinct layers or strata is provided in which the outer surface is of glass hardness and has a fine clear chill, and 15 the second layer or stratum having a comparatively soft fibrous structure which is tough and very strong.

The advantages of our invention will be apparent to those skilled in the art. By our 20 improved method of treating the steel the advantages of the very hard supercarburized steel are retained, while the wearing surface of the steel is changed from a coarsely crystalline structure to a fine clear 25 chill structure of the nature of tool steel which permits of tempering to the required degree of hardness, while increasing the strength and wearing qualities of this outer surface and providing a surface which will 30 not readily spawl off or crack when in use. The soft fibrous layer of steel affords great strength and in this way a hardened supercarburized steel not heretofore known is provided.

35 Modifications may be made in the manner of carrying out the steps comprising our im-

proved method without departing from our invention.

We claim:—

1. The method of treating supercarburized steel consisting in decarburizing for a portion of the depth of supercarburization, removing a portion of the decarburized surface of the steel and then hardening the so-treated steel. 40

2. The method of treating steel having a supercarburized face portion, consisting in decarburizing said face portion, removing part of the decarburized face portion by machining and then hardening the so- 45 treated steel. 50

3. The method of treating supercarburized steel consisting in decarburizing for a portion of the depth of supercarburization, removing a portion of the decarburized surface of the steel by machining and then hardening the so-treated steel. 55

4. The method of treating steel consisting in treating steel having a fibrous portion joined integrally to a supercarburized face portion by decarburizing the supercarburized face for a portion of the depth thereof, removing the decarburized face portion by machining and then water hardening. 60

In witness whereof, we have hereunto set 65 our hands.

WILLIAM H. JONES.  
ANDREW F. MITCHELL.

Witnesses:

ARTHUR J. PARKER,  
E. H. TEWKSBURY.

Copies of this patent may be obtained for five cents each, by addressing the "Commissioner of Patents,  
Washington, D. C."